

# UNITED STATES PATENT OFFICE.

JOHN HERZOG, OF BALTIMORE, MARYLAND.

## COLORED-FIRE COMPOUND.

SPECIFICATION forming part of Letters Patent No. 309,948, dated December 30, 1884.

Application filed October 16, 1884. (Specimens.)

*To all whom it may concern:*

Be it known that I, JOHN HERZOG, a citizen of the United States, residing at Baltimore, in the State of Maryland, have invented a new and useful Improvement in Compositions to be Used as Colored Fire for Tab- leaux, &c., of which the following is a specification.

My invention consists in the addition of vegetable fiber dyed to the color the fire will produce to the ingredients, being combined in the following proportions as instances: Red fire, equal parts of chlorate of potash, nitrate of strontia, and vegetable fiber—such as sawdust—dyed or colored red with aniline, log- wood, or like dye. Green fire, equal parts of chlorate of potash, nitrate baryta, and vegetable fiber dyed with aniline-green. Blue fire, two parts of chlorate of potash, one part blue-

stone, and one part vegetable fiber dyed with 20 blue aniline. These ingredients are to be thoroughly mixed.

By the old way of making colored fire the compounds look all alike—*i. e.*, colorless. By my new process the parties using the fire 25 can tell at a glance the exact color the compound will produce when it is to be burned.

I claim as a new manufacture—

A colored fire comprising the usual chemical ingredients to produce the flame of the de- 30 sired shade, and having in admixture there- with sawdust or like vegetable fiber dyed or stained to a color similar to that which will be produced by the mixture when burned.

JOHN HERZOG.

Witnesses:

W. WILLOUGHBY,  
E. A. NEWMAN.